# EUROPEAN PATENT SPECIFICATION

(11) **EP 1 530 652 B1**
(45) Date of publication and mention of the grant of the patent: **27.04.2011**
(21) Application number: 03784332.3
(22) Date of filing: 22.07.2003
(51) Int. Cl.: C23C 8/00

(54) **WEAR-RESISTANT STAINLESS CUTTING ELEMENT OF AN ELECTRIC SHAVER, ELECTRIC SHAVER**
ABRIEBFESTES ROSTFREIES SCHNEIDELEMENT EINES ELEKTRISCHEN RASIERAPPARATS, EIN ELEKTRISCHER RASIERAPPARAT
ELEMENT COUPANT INOXYDABLE ET RESISTANT A L'USURE DE RASOIR ELECTRIQUE, RASOIR ELECTRIQUE

(30) Priority: 02.08.2002 EP 02078171
(43) Date of publication of application: 18.05.2005
(73) Proprietor: Koninklijke Philips Electronics N.V., 5621 BA Eindhoven (NL)
(72) Inventor: BLAAUW, Hubert, S., NL-5656 AA Eindhoven (NL); DE BEURS, Hans, NL-5656 AA Eindhoven (NL)
(74) Representative: van Wermeskerken, Stephanie Christine
(86) International application number: PCT/IB2003/003179
(87) International publication number: WO 2004/015159

(56) References cited:
- EP-A- 0 506 106
- EP-A- 0 743 144
- EP-A- 1 091 006
- DE-A- 3 431 330
- US-A- 5 953 969
- MELETIS E I ET AL: "LOW-PRESSURE ION NITRIDING OF ALSL 304 AUSTENITIC STAINLESS STEEL WITH AN INTENSIFIED GLOW DISCHARGE" JOURNAL OF VACUUM SCIENCE AND TECHNOLOGY: PART A, AMERICAN INSTITUTE OF PHYSICS. NEW YORK, US, vol. 11, no. 1, 1993, pages 25-33, XP000345530 ISSN: 0734-2101
- PATENT ABSTRACTS OF JAPAN vol. 2000, no. 17, 5 June 2001 (2001-06-05) & JP 01 049594 A (KAIJIRUSHI HAMONO KAIHATSU CENTER:KK), 27 February 1989 (1989-02-27)
- PATENT ABSTRACTS OF JAPAN vol. 010, no. 004 (C-322), 9 January 1986 (1986-01-09) & JP 60 162766 A (KIYUUSHIYUU HITACHI MAKUSERU KK), 24 August 1985 (1985-08-24)
- LEI M K ET AL: "PLASMA SOURCE ION NITRIDING: A NEW LOW TEMPERATURE, LOW-PRESSURE NITRIDING APPROACH" JOURNAL OF VACUUM SCIENCE AND TECHNOLOGY: PART A, AMERICAN INSTITUTE OF PHYSICS. NEW YORK, US, vol. 13, no. 6, 1 November 1995 (1995-11-01), pages 2986-2990, XP000555631 ISSN: 0734-2101
- PATENT ABSTRACTS OF JAPAN vol. 2002, no. 06, 4 June 2002 (2002-06-04) & JP 2002 059319 A (MARUSHO KOGYO KK), 26 February 2002 (2002-02-26)

## Description

The invention relates to a cutting element, as used in an electric shaver, comprising a shaver blade manufactured from maraging or precipitation hardenable stainless steel with a surface hardened by a plasma nitriding hardened layer wherein the plasma nitriding hardened layer consists of a surface top layer of steel, supersaturated with nitrogen, and a diffusion layer adjoining the top layer and having a hardness ranging from a hardness of the top layer to a hardness of the steel before hardening by means of plasma nitriding. The invention also relates to an electric shaver provided with such a cutting element.

Since the introduction of the Philips Coolskin® additive shaver, an electric shaver that can be used with water, and which uses an additive released during operation, it has been found that the stainless steel outer cutting element shows unexpected high wear, leading to customer complaints. It is therefore necessary to provide a more wear-resistant blade, that is, a blade made from a harder material. On the other hand, the blade should not just be sufficiently hard, but also very corrosion-resistant. Corrosion resistance is less of an issue with conventional shavers, but because of the concept of the Coolskin Philishave the blade is in much closer contact with moisture. At present the material used for the manufacture of these cutting elements is stainless maraging steel. This is a steel type with good corrosion resistance qualities but with moderate wear resistance. To increase the hardness, the material is hardened by conventional heat treatment techniques.

Steels that are very well corrosion-resistant are in most cases difficult to harden by heat treatment and have poor tribological properties, with consequent inadequate wear characteristics for the use in the additive shaver mentioned above. The wear of the outer blade is not just caused by contact with the rotating blade inside the shaver head but also through the contact with the skin and hairs which, especially as stubble, can be very though.

The hardness can be further improved by plasma nitriding, as has been demonstrated by patent documents US 5851313 and DE 10039169. In this context also the Japanese document JP 60162766 is relevant. This document discloses the nitriding of a stainless steel or nickel cutting element for achieving a better durability and a less sliding load, for example a better smoothness. According to the Japanese document, only the outside of the blade is simply hardened on one side.

EP-A-0 743 144 discloses a cutting element, as used in an electric shaver, manufactured from maraging or precipitation hardenable stainless steel with a surface hardened by ion-nitriding.

US-A-5,953,969 discloses a screwdriver which has a working end with a surface layer having a hardness of at least 900 HV due to nitriding, wherein an intermediate layer is present between the hard surface layer and a softer region of a core of the working end wherein the hardness decreases with a certain hardness gradient.

DE-A-3431330 discloses a foil blade of an electric shaver made from nickel. The foil blade is covered on one side or on two sides by a hard layer of metal nitride, for example titanium nitride by means of an ion-sputtering process.

The object of the invention is to provide a means to manufacture cutting elements that are both very well corrosion proof and very wear-resistant on all sides.

According to the invention, this object is achieved by a cutting element of the kind referred to in the opening paragraph and characterized in that the thickness of the hardened supersaturated top layer ranges from 5µm to 25µm, and the thickness of the diffusion layer ranges from 5µm to 20µm, wherein the plasma nitriding hardened layer extends over all surfaces of the shaver blade.

Said surface compound layer preferably has a hardness of at least 1300 HV, and in case of austenitic stainless steel at least 1100 HV. The solution provided by the present invention is to comprehensively plasma nitride the cutting element, that is on all sides, de facto giving the entire blade an outer layer of hardened material, making it better wear-resistant on all sides where wear could possibly occur. The advantage of the presence of the diffusion layer is that it additionally strengthens the base material and supports the load-bearing capacity of the compound layer. With a cutting element is meant an individually working shaver blade or a shaver blade that works in cooperation with another shaver blade. Such a construction of cooperating shaver blades can for instance be found in a shaver with an internal rotating cutting element that is surrounded by an external counter cutting element (cap) that has a stationary position. Both the internal rotating cutting element and the external stationary counter cutting element are referred to in this document as cutting elements.

In a preferred embodiment the hardness of the hardened supersaturated top layer is at least 1300 HV, and in case of austenitic stainless steel at least 1100 HV. The cutting element can be designed for use in a shaver of the dry shaver type or for use in a shaver of the additive shaver type.

The invention also relates to an electric shaver provided with a cutting element as disclosed. Such a shaver has the advantages as already mentioned in relation to the cutting element according the invention.

In a method of production of a cutting element according to the invention, the cutting element is formed of austenitic stainless steel after the forming of which the cutting element is hardened by nitriding. Such a method is known from JP-A-62207241 wherein only the faces adjacent to the cutting edge of the cutting element are hardened through a nitride agent. In a method of production of a cutting element according to the invention, the hardening is executed by means of plasma nitriding to a hardness of the top layer of at least 1100 HV and the hardening is executed over all surfaces of the cutting element.

The method enables the manufacture of shaver components out of not hardened (austenitic) stainless steel, which components are hardened later in the production process by inward growth of a hard and wear-resistant compound top layer, thus simplifying the production process. The non-hardened stainless steel can relatively easy be processed. Another problem encountered in the process of manufacturing the cutting elements for the Coolskin® type shaver according to the prior art is that the hardenable steel used according to the prior art for producing shaver heads (for example, Sandvik 1RK91 maraging steel used until now for the production of shaver heads) can only be bought from one source. This undesirable situation, both from a logistical and a commercial point of view, is now solved according to the present invention as the method for producing a cutting element according to the invention makes it possible to use hitherto unsuitable (and relatively inexpensive) types of steel for producing the cutting element according to the invention. Nitriding parameters may be: temperature 300°C to 500°C, process time of 5 to 40 hours, nitriding pressure 250 Pa to 550 Pa and a pulsed plasma process.

The present invention will be elucidated herein below with reference to the annexed drawings, in which:
Fig. 1 is a microscopic view of nitrided 1RK91 maraging steel,
Fig. 2 shows a diffusion profile in NPR+ hardened 1RK91 steel,
Fig. 3 is a cross-section of a hardened lamella,
Fig. 4 is a schematic lengthwise section of lamella, stainless maraging steel,
Fig. 5 is a schematic lengthwise section of a lamella of austenitic stainless steel, and
Fig. 6 is a schematic section of a lamella, showing compound layers and diffusion zones.

The present invention provides a cutting element manufactured according to a method comprising hardening stainless maraging steel, which method consists in plasma nitriding of the manufactured cutting element in such a way that the entire surface of the blade consists of a compounds layer of supersaturated steel, below which lies a diffusion layer in which the nitrogen from the compound layer has diffused into the steel, creating a hardness gradient. A cutting element according to the invention has a hardness of around 1500 HV, which is exceptionally high in relation to the prior art.

Besides stainless martensitic maraging steel, austenitic maraging steel is also suitable for use in the manufacture of a shaver head according to the invention. Actually, austenitic stainless steel is preferred because of its greater corrosion resistance compared with martensitic steel, and it is more widely available. With plasma nitriding it can be made sufficiently hard-wearing, and if the nitriding temperature is kept below 450°C the anticorrosive properties of the austenitic steel are not adversely affected.

During the nitriding process, nitrogen penetrates and diffuses into the base material from the outside inwards. In the so-called compound layer the hardness is quite even and the metal structure is supersaturated with nitrogen. The thickness of this layer depends on the duration of the nitriding process. Underneath this layer lies the diffusion zone, in which nitrogen diffuses into the base material, the hardness of which decreases with depth. Figs. 1 and 2 illustrate this phenomenon.

Maraging steel and precipitation-hardenable stainless steel can undergo a precipitation hardening step prior to or together with the plasma nitriding step according to the invention.

As is shown in Fig. 6, the diffusion zones in a lamella of a shaver head according to the invention are nearly meeting or overlapping. The hardness of the outer surface depends on the material used. Fig. 4 shows a hardness of 1500 HV for the compound layer and an average hardness of the diffusion layer of 500 HV. For an austenitic stainless steel, the data are 1400 HV to 1600 HV and above 200 HV, respectively, as is shown in Fig. 5. These values are unusual and hitherto unknown in the state of the art. Since the diffusion zones underneath the compound layers are nearly meeting or even overlapping, the mechanical strength of the lamellae is considerably increased. Hardening of the metal is usually achieved at the cost of toughness. In other words, it becomes more brittle. If the blade were uniformly hardened through and through to a hardness of 1500HV, it would become very brittle and consequently would snap easily. With the process according to the invention this disadvantage is avoided.

As is shown in Fig. 3, which shows a cross-section of a plasma-nitrided lamella, the compound layer is indeed covering the entire surface in an even manner, assuring sufficient wear resistance on all sides. Although with plasma nitriding of intricate shapes it is difficult to achieve an even layer of hardened material (because of which a two-stage process for nitriding is proposed), the present manufacturing process does not suffer from this problem. As can be seen in the cross-section in Fig. 3, an even thickness of the nitrided layer is achieved.

Prior to the nitriding process, the maraging and precipitation hardenable steels must first be hardened by an ageing heat treatment. Optionally this may be combined with the nitriding process as this, according to the present invention, is carried out at the same temperature. The plasma nitriding process employed here is commonly known in the art.

Preferred embodiments.

To better illustrate the present invention two examples are given below, in which stainless maraging steel and austenitic stainless steel, respectively, are used. These examples are strictly non-limitative, as any type of steel with suitable properties may be used.

### Example 1

Manufacture of a shaver head according to the invention from 1RK91 maraging steel.

After manufacture, the cutting element is kept in a pulsed nitriding furnace at 375°C for 20 hours in 475 Pa nitrogen gas pressure, during which the nitriding takes place. With an average thickness of the lamella of around 70µm this results in a compound layer of around 10 to 20 µm. As can be seen in the schematic representation in Fig. 6, the diffusion zones just touch. In the case of 1RK91 steel, the hardness of originally 500 HV has been increased to 1500 HV on the outside of the compound layer. Also the Young modulus increases in the compound layer by 23%, rising from 177 GPa to 217 GPa.

### Example 2

This proceeds in an analogous manner to example 1, but with the use of AISI 316 austenitic steel. The chosen temperature is 425°C. The resulting hardness ranges from the original 200 HV in the center core of the lamella to 1400 HV on the outside surface.

Thus it is shown that a variety of steels can be hardened by plasma nitriding to obtain a desired hardness of around 1500 HV. In either case the corrosion resistance was not impaired.

## Claims

1. Cutting element, as used in an electric shaver, comprising a shaver blade manufactured from maraging or precipitation hardenable stainless steel or austenitic stainless steel with a surface hardened by a plasma nitriding hardened layer, wherein the plasma nitriding hardened layer consists of a surface top layer of steel, supersaturated with nitrogen, and a diffusion layer adjoining the top layer and having a hardness ranging from a hardness of the top layer to a hardness of the steel before hardening by means of plasma nitriding, **characterised in that** the thickness of the hardened supersatured top layer ranges from 5µm to 25µm, and the thickness of the diffusion layer ranges from 5µm to 20µm, wherein the plasma nitriding hardened layer extends over all surfaces of the shaver blade.

2. Cutting element according to claim 1, **characterised in that** the hardness of the hardened supersaturated top layer is at least 1300 HV.

3. Cutting element according to any of the foregoing claims, **characterised in that** the cutting element is for use in a shaver of the dry shaver type.

4. Cutting element according to any of the claims 1 - 2, **characterised in that** the cutting element is for use in a shaver of the additive shaver type.

5. Electric shaver comprising at least one of the cutting elements according any of the claims 1 - 4.

## Patentansprüche

1. Schneidelement, wie in einem elektrischen Rasierapparat verwendet, mit einem Schermesser, das aus martensitaushärtendem oder ausscheidungshärtendem, rostfreiem Stahl oder austenitischem, rostfreiem Stahl hergestellt wird, mit einer durch eine durch Plasmanitrieren gehärtete Schicht gehärteten Oberfläche, wobei die durch Plasmanitrieren gehärtete Schicht aus einer oberen Oberflächenschicht aus Stahl, mit Stickstoff übersättigt, und einer Diffusionsschicht, die an die obere Schicht angrenzt und eine Härte aufweist, die im Bereich von einer Härte der oberen Schicht bis zu einer Härte des Stahls vor Härten durch Plasmanitrieren liegt, besteht, **dadurch gekennzeichnet, dass** die Dicke der gehärteten, übersättigten, oberen Schicht im Bereich von 5 µm bis 25 µm und die Dicke der Diffusionsschicht im Bereich von 5 µm bis 20 µm liegt, wobei die durch Plasmanitrieren gehärtete Schicht sich über sämtliche Oberflächen des Schermessers erstreckt.

2. Schneidelement nach Anspruch 1, **dadurch gekennzeichnet, dass** die Härte der gehärteten, übersättigten, oberen Schicht mindestens 1300 HV beträgt.

3. Schneidelement nach einem der vorangegangenen Ansprüche, **dadurch gekennzeichnet, dass** das Schneidelement zur Verwendung in einem Rasierapparat, Typ Trockenrasierer, dient.

4. Schneidelement nach einem der Ansprüche 1-2, **dadurch gekennzeichnet, dass** das Schneidelement zur Verwendung in einem Rasierapparat, Typ Additive Shaver, dient.

5. Elektrischer Rasierapparat mit mindestens einem der Schneidelemente nach einem der Ansprüche 1-4.

## Revendications

1. Elément coupant tel qu'utilisé dans un rasoir électrique, comprenant une lame de rasoir fabriquée en acier inoxydable durcissable par maraging ou précipitation ou en acier inoxydable austénitique avec une surface durcie par une couche durcie par nitruration au plasma, dans lequel la couche durcie par nitruration au plasma consiste en une couche supérieure de surface en acier, sursaturée en azote, et une couche de diffusion attenante à la couche supérieure et présente une dureté allant d'une dureté de la couche supérieure à une dureté de l'acier avant durcissement au moyen d'une nitruration au plasma, **caractérisé en ce que** l'épaisseur de la couche supérieure sursaturée durcie va de 5 µm à 25 µm, et l'épaisseur de la couche de diffusion va de 5 µm à 20 µm, la couche durcie par nitruration au plasma s'étendant sur toutes les surfaces de la lame de rasoir.

2. Elément coupant, selon la revendication 1, **caractérisé en ce que** la dureté de la couche supérieure sursaturée durcie est d'au moins 1300 HV.

3. Elément coupant, selon l'une quelconque des revendications précédentes, **caractérisé en ce que** l'élément de coupe est destiné à une utilisation dans un rasoir du type rasoir sec.

4. Elément coupant, selon l'une quelconque des revendications 1 à 2, **caractérisé en ce que** l'élément de coupe est destiné à une utilisation dans un rasoir de type rasoir additif.

5. Rasoir électrique, comprenant au moins un des éléments coupants selon l'une quelconque des revendications 1 à 4.
